

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## STAIN RESISTING COBALT ALLOY

No Drawing.

Application filed April 29, 1930. Serial No. 448,429.

This invention relates to stain resisting alloys containing as essential constituents the metals iron, chromium, manganese and cobalt.

5 In application serial No. 435,957 filed by me on March 14, 1930, I have disclosed stain resisting ferrous alloys containing not less than about sixteen per cent nor more than about twenty-two per cent of chromium, 10 and not less than about six per cent nor more than about sixteen per cent of manganese. I have shown that when these alloys contain not more than about three tenths per cent carbon and preferably not more than twelve hundredths per cent of this 15 element, they possess excellent workability and are adapted to deep drawing operations. In application Serial No. 448,428 filed simultaneously herewith I have shown that the iron-chromium-manganese compositions are more resistant than the workable stain resisting iron-chromium-nickel alloys to attack by gasses containing sulphur compounds and I have also shown that an addition of cobalt to the iron-chromium-manganese base will markedly increase its strength at elevated temperatures without destroying its working properties or its resistance to 20 sulphur-bearing gases and other corrosive influences. The invention claimed herein is the group of alloys produced by so combining iron, chromium, manganese and cobalt.

25 The high temperature strength is increased by cobalt percentages as low as one per cent and perhaps even lower. With higher percentages of cobalt the effect is more pronounced but as the cobalt rises 30 above about five per cent the high temperature strength is not additionally greatly increased. Cobalt percentages between the approximate limits of one per cent and ten per cent are regarded as the most useful. 35 The following examples show the effect

of cobalt on the strength of the chrome-iron-manganese alloys at 900° C.

| Percent Cr | Percent Mn | Percent C | Percent Co | Lbs./sq. in. max. stress | Percent el. in 2" | Percent red. of area | 50 |
|------------|------------|-----------|------------|--------------------------|-------------------|----------------------|----|
| 17.17      | 8.09       | 0.06      | -----      | 9,250                    | 43                | 66.50                |    |
| 17.19      | 10.27      | 0.11      | -----      | 9,000                    | 43                | 72.90                |    |
| 17.38      | 8.60       | 0.09      | 2.45       | 14,500                   | 44                | 72.80                |    |
| 18.50      | 8.80       | 0.12      | 4.97       | 19,120                   | 36                | 73.50                |    |
| 17.36      | 8.76       | 0.14      | 8.85       | 18,250                   | 45                | 65.40                | 55 |
| 17.56      | 8.74       | 0.15      | 13.95      | 21,400                   | 25                | 65.10                |    |

In the tests tabulated above the test pieces were held at 900° C. for about forty minutes before applying the load and the load 60 was applied gradually and at a uniformly increasing rate so that about twenty minutes was required to rupture the test piece.

The following examples show the effect of cobalt on the strength of the chrome-65 iron-manganese alloys at 600° C.

| Percent Cr | Percent Mn | Percent C | Percent Co | Lbs./sq. in. |             | Percent el. in 2" | Percent red. of area | 70 |
|------------|------------|-----------|------------|--------------|-------------|-------------------|----------------------|----|
|            |            |           |            | Yield point  | Max. stress |                   |                      |    |
| 17.17      | 8.09       | 0.06      | -----      | 18,000       | 33,750      | 39                | 74.10                |    |
| 17.19      | 10.27      | 0.11      | -----      | 20,000       | 39,750      | 41                | 74.30                |    |
| 17.38      | 8.60       | 0.09      | 2.45       | 23,300       | 47,100      | 34                | 71.60                |    |
| 18.50      | 8.80       | 0.12      | 4.97       | 26,000       | 50,500      | 35                | 65.80                | 75 |
| 17.36      | 8.76       | 0.14      | 8.85       | 27,000       | 57,750      | 38                | 60.80                |    |
| 17.56      | 8.74       | 0.15      | 13.95      | 29,000       | 59,000      | 34                | 51.10                |    |

The results of the tests at 600° C. show clearly that the addition of cobalt greatly increases the yield point of these alloys, 80 high yield point being recognized as a desirable property in alloys subjected to high temperatures over long periods.

If a high degree of workability is not 85 essential, as when the alloy is to be used in the form of a casting, the carbon content may rise beyond the limits mentioned above. While increasing carbon content may somewhat impair the stain resisting properties 90 of the metal, alloys containing at least one

per cent carbon have a distinct field of utility. Where the alloy is to be subjected to deep drawing or like severe cold working operation it is often advantageous to cool it in air or quench it from temperatures in the vicinity of 1000° C. to 1150° C.

A principal field of application for the herein described alloys is in the thermal decomposition of hydrocarbon material, for example the cracking of petroleum fractions to produce gasoline. Such decompositions are ordinarily carried out in tubes and the latter may be subjected at a high temperature to oxidizing conditions on the outside and simultaneously to the action of sulfur compounds associated with the material being cracked and contained within the tubes. The alloys of the invention are in all respects admirably adapted to the fabrication of tubes for such operations, and they are equally suitable for making the tubular condensers in which the cracked products are usually liquefied.

I claim:

25 1. A ferrous alloy containing chromium not less than about sixteen percent nor more than about twenty-two per cent, manganese not less than about six per cent nor more than about sixteen per cent and cobalt not less than about one per cent nor more than about ten per cent, and carbon, the carbon content being, not more than three tenths of one per cent; the remainder being chiefly iron.

30 2. A stain resisting ferrous alloy having deep drawing properties and containing chromium about eighteen percent, manganese about eight per cent, carbon, the content of carbon being, not more than twelve hundredths per cent and about five per cent of cobalt; the remainder being chiefly iron.

35 3. An article of manufacture subject to the action of hot sulfur-bearing gases, said article being composed of a ferrous alloy containing chromium not less than about 45 16% and not more than about 22%, manganese not less than about 6% and not more than about 16%, cobalt not less than 1% and not more than about 10%, and carbon, the carbon content being not more than about 50 0.3%; the remainder being chiefly iron.

40 4. An oil cracking tube composed of a ferrous alloy containing chromium not less than about 16% and not more than about 22%, manganese not less than about 6% and not more than about 16%, cobalt not less than about 1% and not more than about 10%, and carbon, the carbon content being not more than about 0.3%; the remainder being chiefly iron.

45 5. An oil cracking tube composed of a ferrous alloy containing chromium not less than about 16% and not more than about 22%, manganese not less than about 6% and not more than about 16%, cobalt not less than about 1% and not more than about 10%, and carbon, the carbon content being not more than about 0.3%; the remainder being chiefly iron.

10%, and carbon, the carbon content being not more than about 0.12%; the remainder being chiefly iron.

In testimony whereof, I affix my signature.

FREDERICK M. BECKET. 70

75

80

85

90

95

100

105

110

115

120

125

130